



US008048196B2

(12) **United States Patent**  
**Reichel**

(10) **Patent No.:** **US 8,048,196 B2**  
(45) **Date of Patent:** **Nov. 1, 2011**

(54) **METHOD AND DEVICE FOR PRODUCING STAINLESS STEEL WITHOUT USING A SUPPLY OF ELECTRICAL ENERGY, BASED ON PIG-IRON THAT HAS BEEN PRE-TREATED IN A DDD INSTALLATION**

(75) Inventor: **Johann Reichel**, Düsseldorf (DE)

(73) Assignee: **SMS Siemag Aktiengesellschaft**, Düsseldorf (DE)

(\*) Notice: Subject to any disclaimer, the term of this patent is extended or adjusted under 35 U.S.C. 154(b) by 0 days.

(21) Appl. No.: **12/312,888**

(22) PCT Filed: **Nov. 20, 2007**

(86) PCT No.: **PCT/EP2007/010013**

§ 371 (c)(1),

(2), (4) Date: **Jul. 20, 2009**

(87) PCT Pub. No.: **WO2008/064798**

PCT Pub. Date: **Jun. 5, 2008**

(65) **Prior Publication Data**

US 2010/0024600 A1 Feb. 4, 2010

(30) **Foreign Application Priority Data**

Nov. 30, 2006 (DE) ..... 10 2006 056 671

(51) **Int. Cl.**

**C21B 13/14** (2006.01)

**C21C 7/064** (2006.01)

**C21C 7/068** (2006.01)

(52) **U.S. Cl.** ..... **75/458; 75/551; 75/552; 75/569**

(58) **Field of Classification Search** ..... **75/458, 75/551, 552, 569**

See application file for complete search history.

(56)

**References Cited**

**U.S. PATENT DOCUMENTS**

|                |        |                          |
|----------------|--------|--------------------------|
| 3,231,369 A    | 1/1966 | Gorlich et al.           |
| 7,998,243 B2 * | 8/2011 | Rose et al. ..... 75/551 |

**FOREIGN PATENT DOCUMENTS**

|    |             |         |
|----|-------------|---------|
| DE | 1 508 284   | 5/1970  |
| DE | 2 014 339   | 10/1970 |
| DE | 196 21 143  | 8/1997  |
| EP | 1 310 573   | 5/2003  |
| WO | 02/075003   | 9/2002  |
| WO | 03/106716   | 12/2003 |
| WO | 2006/050963 | 5/2006  |

\* cited by examiner

*Primary Examiner* — George Wyszomierski

*Assistant Examiner* — Tima M McGuthry Banks

(74) *Attorney, Agent, or Firm* — Lucas & Mercanti, LLP;  
Klaus P. Stoffel

(57) **ABSTRACT**

The aim of the invention is to produce stainless steel for all stainless steel products both in the austenitic and the ferritic range, based on liquid pig-iron and FeCr solids, without using a supply of electrical energy. According to the invention, the liquid pig-iron, after being pre-treated in a blast furnace (1), is subjected to a DDD treatment (dephosphorization, desilicization and desulphurization), is heated, finished or alloyed and deoxidized. The quantity of slag-free liquid pig-iron that has been pre-treated in the blast furnace (1) and a DDD device (2) is separated and introduced into two classic “twin” AOD-L converters (3, 4), where the required chemical process steps (of the heating, decarburization and alloying stages) take place in parallel contrary processes using autonomous chemical energy, the heating stage being carried out first in the first twin AOD-L converter (3) and the decarburization being carried out first in the second twin AOD-L converter (4).

**7 Claims, 1 Drawing Sheet**



*Fig. 1**Fig. 2*

## 1

**METHOD AND DEVICE FOR PRODUCING  
STAINLESS STEEL WITHOUT USING A  
SUPPLY OF ELECTRICAL ENERGY, BASED  
ON PIG-IRON THAT HAS BEEN  
PRE-TREATED IN A DDD INSTALLATION**

The present application is a 371 of international application PCT/EP2007/010013 filed Nov. 20, 2007, which claims priority of DE 10 2006 056671.8, filed Nov. 30, 2006, the priority of these applications is hereby claimed and these applications are incorporated herein by reference.

**BACKGROUND OF THE INVENTION**

The present invention relates to a method and a device for stainless steel production without electrical energy supply on the basis of liquid pig-iron and FeCr solids, wherein, after a pretreatment in a blast furnace and a DDD treatment (dephosphorization, desiliconization, desulphurization) in a DDD installation, the liquid pig-iron is subsequently heated, refined or alloyed in an AOD converter, is reduced and finally an adaptation/adjustment of the treated steel melt is carried out in a ladle furnace.

The use of an AOD converter for manufacturing noble steels is already known. Thus WO 02/075003 describes a control method based on a continuous measurement of exhaust gases in combination with a computer and a dynamic model by means of which the necessary blow rates of oxygen and inert gas as well as the material charges are controlled.

EP 1 310 573 A2 discloses a method for manufacturing a metal melt, particularly for quenching a metal melt for manufacturing, for example, alloyed stainless steel or noble steel in an AOD converter, wherein the method is based on a computer technology which takes place in accordance with a processed model and which controls the metallurgical installation, the process model describes the behavior for at least one variable process parameter between a first process value, an adjusting value, and a final process value. An example describes the process sequence for manufacturing a steel of the class AISI 304.

Stainless steels of the ferritic steel group AISI 4xx are conventionally always manufactured from scrap of the same type in the EAF and are later additionally alloyed and decarbonized in the AOD converter. In order to utilize the use of pig-iron, pig-iron pretreated in a steel mill with scrap and alloy melted into the pig-iron is mixed in a ladle outside of the furnace and is then charged into the converter.

WO 2006/050963 A2 proposes a method for producing stainless steel of the ferritic steel group AISI 4xx, particularly the steel group AISI 430, on the basis of liquid pig-iron and FeCr solids, with a DDD process line and the AOD converter with successively carried out method steps:

Pretreatment of the liquid pig-iron in the blast furnace, DDD treatment of the pig-iron in a suitable DDD installation, and charging the AOD converter with slag-free liquid pig-iron,

Heating, refining/alloying, and reducing the liquid pig-iron in the AOD converter,

Final adaptation/adjustment of the treated steel melt in the casting ladle.

In this known method, the manufacture of the stainless steel is carried out advantageously with the use of the AOD converter without the use of an EAF, i.e., without the supply of electrical energy. However, this known method has the

## 2

disadvantage that finally, because of the lack of energy in this method, only the manufacture of ferritic steels is possible.

**SUMMARY OF THE INVENTION**

Starting from this prior art, the object of the invention resides in utilizing the method known from WO 2006/050963 A2 with AOD technology for directly charging the pig-iron and subsequent alloying in the converter for the production of stainless steel of all stainless qualities in the austenitic as well as in the ferritic range with the use of autogenic chemical energy.

The above object for manufacturing stainless steel of the mentioned steel quality is solved in that, for the stainless steel production of all stainless qualities in the austenitic range as well as in the ferritic range, the slag-free liquid pig-iron quantity pretreated in the blast furnace and in a DDD installation is separated and introduced into two classic "Twin" AOD-L converters, in which the required chemical process steps (heating, decarbonizing, and alloying) are carried out with the use of autogenic chemical energy in a parallel contrary sequence with the use of autogenic chemical energy, wherein charging and heating are initially carried out in the first Twin AOD-L converter and decarbonization is initially carried out in the second Twin AOD-L converter.

After concluding the DDD treatment in an external DDD installation, a deslagging of the pig-iron is necessary prior to the subsequent heating in the converter, because the typical AOD process is supposed to start slag-free. This also increases the efficiency of the single-hole lance which is used in the second AOD-converter and a free surface of the melt is ensured for soaking the process gases.

Heating of the pig-iron to a desired temperature or a temperature which is required for the subsequent process steps takes place by Si-oxidation. For this purpose, FeSi is charged into the Twin AOD-L converter and an oxygen/inert gas mixture is blown through the side nozzles of a top lance into and onto the pig-iron. For this purpose, a three-hole top lance or four-hole top lance known from BOF blowing technology (treatment of C steels) is used in the first Twin AOD-L converter, and a single-hole top lance typical for the AOD-L process is used in the second AOD-L converter.

Since heating of the initial metal is carried out according to the invention after the DDD treatment, it is especially possible to charge Ni or Ni-alloys into the Twin AOD-L converters. In this manner, the balance energy can be carried out in any chosen manner.

Because of the contrary sequence of the process steps carried out at different times in the two Twin AOD-L converters, decarbonization and alloying of the melt takes place in the first Twin AOD-L converter after the conclusion of heating of decarbonization at alloying, while in the second Twin AOD-L converter, after conclusion of the classical decarbonization and/or treatment steps belonging thereto (such as, for example, desulphurization and alloying including tapping), the pig-iron is charged and heated.

Because of the separation of the pretreated slag-free liquid pig-iron quantity according to the invention into two Twin AOD-L converters arranged in parallel in the process line after the blast furnace and the DDD installation, and because the process steps are carried out in the converters in a contrary manner, the production of all RST steel qualities is facilitated in an advantageous manner. Simultaneously, a decoupling of the requirement of electrical energy for all qualities takes place because the only energy carrier used is the autogenic chemical energy already present in the pig-iron and introduced through the charged FeSi. Moreover, this separation of

the pig-iron quantity and the process pattern, a reliable temperature pattern, reduced process costs as well as reduced investment costs are achieved because always only a small pig-iron quantity has to be treated at a given time.

In the following, the method according to the invention will be explained in more detail with the aid of schematic drawing figures.

#### BRIEF DESCRIPTION OF THE DRAWINGS

In the drawing:

FIG. 1 is a process line showing an example,

FIG. 2 shows the contrary process pattern in two Twin AOD-L converters.

#### DETAILED DESCRIPTION OF THE INVENTION

In FIG. 1, a drawing figure illustrates an example of a process line for the manufacture of stainless steel. After emerging from the blast furnace 1 and a DDD treatment in a DDD installation 2, the liquid pig-iron quantity is divided and introduced into two Twin AOD-L converters 3, 4 which are arranged in parallel. In the converters, in a contrary sequence of the process steps, a temperature increase takes place as required by the Si-oxidation and the refinement and alloying of the liquid pig-iron. After the treatment in the Twin AOD-L converters 3, 4, the steel melt from the two Twin AOD-L is brought together in a ladle 5 and is brought for the final adaptation/adjustment in the ladle furnace 6 and to the casting machine 7.

FIG. 2 shows the contrary sequence of the process steps carried out in the Twin AOD-L converters 3 and 4. While charging and heating V8 of the pig-iron pretreated in the blast furnace 1 and a DDD installation 2 are started in the Twin AOD-L converter 3 (on the left hand side in the drawing) of the pig-iron pretreated in the blast furnace 1 and a DDD installation 2, with subsequent AOD treatment V9 with decarbonization and alloying for producing, for example, AISI 3xx, 4xx, 2xx stainless steel qualities; simultaneously, in the Twin AOD-L converter 4 (shown on the right hand in the drawing), initially the AOD treatment V9 is carried out and only then charging and heating V8 of the pig-iron are carried out.

The selected illustration in FIG. 1 has the purpose of particularly clearly emphasizing that the same method steps are not carried out simultaneously at any time in the converters 3, 4, on which are based the division of the method in two converters providing the process-technological advantage of the invention which is the separation of the method into two converters. In other words, charging and heating in the converter 3 is synchronized with the AOD-L treatment in the converter 4 and vice versa. The AOD-L treatment in the converter 3 is synchronized with the charging and heating steps in the converter 4.

#### LIST OF REFERENCE NUMERALS

- 1 Blast Furnace/BF
- 2 DDD Installation
- 3,4 Twin AOD-L Converter
- 5 Ladle/CL
- 6 Ladle Furnace/LF
- 7 Casting Machine/CCM

#### Process Steps

- V8 Charging and heating of the pretreated pig-iron
- V9 Decarbonizing and alloying (AOD treatment)

I claim:

1. Method for stainless steel production without electrical energy supply based on liquid pig-iron and FeCr solids, wherein, after a pretreatment in a blast furnace (1) and a DDD treatment (dephosphorization, desiliconization, desulphurization) in a DDD installation (2), the liquid pig-iron is subsequently heated, refined or alloyed, reduced in an AOD (Argon Oxygen Decarburization) converter (3, 4), and subsequently an adaptation/adjustment of the treated steel melt in a ladle furnace (5) is carried out, wherein, for stainless steel production of all stainless qualities in the austenitic range as well as in the ferritic range a slag-free liquid pig-iron quantity pretreated in a DDD installation (2) is separated and introduced into two classical Argon Oxygen Decarburization with Lance (AOD-L) converters (3, 4) that carry out, in a parallel contrary sequence, the necessary chemical process steps of heating (V8), and decarbonizing and alloying (V9) using autogenous chemical energy, wherein initially charging and heating (V8) are carried out in the first AOD-L converter (3) and decarbonization (V9) is initially carried out in the second AOD-L converter (4).

2. Method according to claim 1, wherein an Si-oxidation is carried out for heating (V8) of the pig-iron, for which purpose the pig-iron is charged with FeSi.

3. Method according to claim 2, wherein decarbonization and alloying (V9) of the melt are carried out in the first AOD-L converter (3) after the conclusion of charging and heating (V8).

4. Method according to claim 3, wherein, for carrying out the Si-oxidation, an oxygen/inert gas mixture is blown into and onto the pig-iron in the first AOD-L converter (3).

5. The method according to claim 2, wherein, in the second AOD-L converter (4), after the conclusion of decarbonization (V9) and all related treatment steps, including desulphurization and alloying including tamping, the pig-iron is charged and heated.

6. The method according to claim 5, wherein, for carrying out the Si-oxidation in the second AOD-L converter (4), an oxygen/inert gas mixture is blown into and onto the pig-iron through side nozzles and a top lance.

7. The method according to claim 1, wherein equal quantities of pig-iron are introduced into the two AOD-L converters (3, 4).

\* \* \* \* \*